

Patented Nov. 27, 1928.

1,692,950

## UNITED STATES PATENT OFFICE.

PAUL ONNERTZ, OF BERLIN-WILMERSDORF, AND BENNO SCHWÄRZEL, OF BERLIN, GERMANY, ASSIGNEES, BY MESNE ASSIGNMENTS, TO GRASSELLI DYESTUFF CORPORATION, OF NEW YORK, N. Y., A CORPORATION OF DELAWARE.

### PROCESS FOR PROTECTING ANIMAL FIBER.

No Drawing. Application filed June 22, 1925, Serial No. 38,901, and in Germany August 21, 1924

In U. S. Patent No. 1,419,497 there is described a process for protecting animal fiber under treatment with alkaline liquids which consists in adding to the alkaline liquid sugar or sulphite cellulose liquor or the active constituents thereof or both sugar and sulphite cellulose liquor or the active constituents thereof.

We have now found that the sulphurized phenols, which form a slightly yellow colored solution with an aqueous sodium carbonate solution such as are obtainable by treating phenols with sulphur in strong sulphuric acid or with sulphur chloride (see French Patent No. 537,207, British Patent No. 13,657/1913, German Patents Nos. 362,383 and 410,973, etc.) have an effect similar to that of sugar and that of sulphite cellulose liquor or its active constituents for the purpose in question.

The following examples illustrate the invention without limiting it, the parts being by weight:

1. 25 grams of woolen yarn are treated for 25 half an hour at 40° C. in a bath consisting of 1 litre of water, 10 grams of crystallized sodium sulphide and 5 grams of the solid colorless sodium compound of the sulphurized product obtainable from chlorophenol. 30 The wool is then washed and treated with dilute acetic acid for neutralizing any residual alkali; it is then again washed and dried. During this treatment the woolen yarn does not lose either in strength or in elasticity as 35 is shown by tests made on the Schopper-testing-machine whereas when wool is submitted to the same treatment but with omission of the sulphurized chlorophenol the extensibility is diminished by 38% and the tensile 40 strength by 46%.

2. 25 grams of woolen yarn are treated for half an hour at 75-80° C. in a bath consisting of 1 litre of water, 15 grams of anhydrous sodium carbonate and 5 grams of the sodium 45 compound of the product of the reaction of sulphur and strong sulphuric acid on phenol

at a high temperature. The wool is then washed, acidified with acetic acid, washed and dried. The yarn so treated retains its texture, elasticity and strength whereas wool subjected to a like treatment without a protective agent has a harder texture and shows a loss of about 9 per cent of its extensibility and about 23 per cent of its tensile strength.

What we claim is,—

1. The method of protecting animal fibers from the injurious effect of alkaline liquids, which comprises treating the fibers with an alkaline liquid in the presence of a sulphurized phenol which does not possess the properties of a dyestuff and which is soluble in a sodium carbonate solution with only a slight color.

2. The method of protecting animal fibers from the injurious effect of alkaline liquids, which comprises treating the fibers with an alkaline liquid in the presence of a sulphurized phenol, obtainable by treating phenols with sulphur and strong sulphuric acid.

3. The method of protecting animal fibers from the injurious effect of alkaline liquids, which comprises treating the fibers with an alkaline liquid in the presence of the sodium derivative of a sulphurized phenol, obtainable by treating phenols with sulphur and strong sulphuric acid at a high temperature.

4. The method of protecting animal fibers from the injurious effect of alkaline liquids, which comprises treating animal fibers with an alkaline liquid containing an alkaline compound and a sulphurized phenol, said sulphurized phenol being soluble in an aqueous sodium carbonate solution with a slightly yellow color, the weight of sulphurized phenol in said alkaline liquid being about one-third of the weight of alkaline compound in said alkaline liquid.

In testimony whereof we affix our signatures.

DR. PAUL ONNERTZ.  
DR. BENNO SCHWÄRZEL.